



US005879847A

# United States Patent [19]

Yoshinaga et al.

[11] Patent Number: **5,879,847**[45] Date of Patent: **\*Mar. 9, 1999**

[54] **ELECTROPHOTOGRAPHIC PHOTOSENSITIVE MEMBER, A PROCESS-CARTRIDGE INCLUSIVE THEREOF AND AN IMAGE FORMING APPARATUS**

[75] Inventors: **Kazuo Yoshinaga**, Kawasaki; **Yuichi Hashimoto**, Tokyo; **Shunichiro Nishida**, Yokohama, all of Japan

[73] Assignee: **Canon Kabushiki Kaisha**, Tokyo, Japan

[\*] Notice: This patent issued on a continued prosecution application filed under 37 CFR 1.53(d), and is subject to the twenty year patent term provisions of 35 U.S.C. 154(a)(2).

[21] Appl. No.: **944,981**

[22] Filed: **Oct. 7, 1997**

## Related U.S. Application Data

[63] Continuation of Ser. No. 744,181, Nov. 5, 1996, abandoned.

## Foreign Application Priority Data

Nov. 6, 1995 [JP] Japan ..... 7-287693

[51] **Int. Cl.<sup>6</sup> G03G 5/47**

[52] **U.S. Cl. 430/67; 430/66; 399/111**

[58] **Field of Search 430/66, 67; 399/111**

## References Cited

### U.S. PATENT DOCUMENTS

3,957,725 5/1976 Limburg ..... 260/46.5 R  
5,230,976 7/1993 Schank et al. ..... 430/59  
5,232,801 8/1993 Rule et al. ..... 430/59

5,326,661 7/1994 Sansone et al. ..... 430/20  
5,591,551 1/1997 Audett et al. ..... 430/18

## FOREIGN PATENT DOCUMENTS

0224784 6/1987 European Pat. Off. ..... C08G 77/38  
446895 9/1991 European Pat. Off. ..... C07F 7/10  
0457212 11/1991 European Pat. Off. ..... C08F 7/08  
57-030843 2/1982 Japan ..... G03G 5/14  
61-132594 6/1986 Japan ..... G03G 5/05  
4-324454 11/1992 Japan ..... G03G 5/147

## OTHER PUBLICATIONS

Noll, W., "Preparation of Polyorganosiloxanes," Chemistry and Technology of Silicones, Chapter 5, pp. 190-245 (1968).

Database WPI, Section Ch., Week 8036, Derwent; Class E11, AN-80-62981C for JP 55 095 953 A (1980).

Primary Examiner—John L. Goodrow  
Attorney, Agent, or Firm—Fitzpatrick, Cella, Harper & Scinto

## [57] ABSTRACT

The present invention provides an electrophotographic photosensitive member having a substrate and a photosensitive layer thereupon, wherein a surface protecting layer of the photosensitive member contains a resin which is obtained by curing a curable organosilicon polymer and an organosilicon-modified positive hole transporting compound; a process-cartridge which has, in addition to the electrophotographic photosensitive member, at least one from among a primary charging means, a developing means, and a cleaning means placed into a housing, and which can be reversibly mounted to an image forming apparatus; and the image forming apparatus using the electrophotographic photosensitive member.

**22 Claims, 6 Drawing Sheets**

FIG. 1



FIG. 2





FIG. 4



FIG. 5



FIG. 6



FIG. 7



FIG. 8



**ELECTROPHOTOGRAPHIC  
PHOTOSENSITIVE MEMBER, A PROCESS-  
CARTRIDGE INCLUSIVE THEREOF AND AN  
IMAGE FORMING APPARATUS**

This application is a continuation of application Ser. No. 08/744,181 filed Nov. 5, 1996, now abandoned.

**BACKGROUND OF THE INVENTION**

1. Field of the Invention

This invention relates to an electrophotographic photosensitive member having a specific surface coat thereupon, a process cartridge containing the photosensitive member, and an image forming apparatus.

2. Related Background Art

The surface of an electrophotographic photosensitive member must be sufficiently durable, because mechanical and electric forces involved in the operation of a charging means, developing means, transferring means and cleaning means are often imposed upon it from outside.

To be more explicit, the surface must be sufficiently durable to withstand wear and damages due to friction, and deteriorating effects by ozone often generating in association with corona charging at high humidity. Further, it is often exposed to toner dusts scattered by repeated developing and cleaning. Therefore, the surface of the photosensitive member must be provided with improved cleaning property.

To provide the surface of the photosensitive member with properties to cope with above problems, surface protective layers containing various resins as their main ingredients have been tried. For example, Japanese Patent Application Laid-Open No. 57-30843 proposes a protective coat whose resistance to wear and electric resistance are controlled by the addition of metal oxide particles to act as electro-conductive particles.

Besides, studies have been made to improve the physical properties of the surface of the photosensitive member by adding various materials thereto. Such materials include, to take silicone compounds as an example which have been known to have a low surface energy, silicone oil (Japanese Patent Application Laid-Open No. 61-132954), polydimethylsiloxane, silicone resin powders (Japanese Patent Application Laid-Open No. 4-324454), cross-linked silicone resins, poly(carbonate-silicon) block copolymers, silicon-modified polyurethanes, and silicon-modified polyesters.

The representative polymers which have a low surface energy include fluorine polymers which are represented further by polytetrafluoroethylene powders and carbon fluoride powders.

A surface protective layer comprising a metal oxide or the like tends to have a big surface energy while having a sufficient hardness, and thus it may cause problems of the cleaning property. The silicone resin, though being excellent in having a small surface energy, is not readily compatible to other resins. Therefore, when such a resin is used in an addition system, it tends to agglutinate to cause light scattering, or to bleed upon the surface to crystallize there, thereby impairing the stability of the product. The fluorine polymer which is known to have a low surface energy is usually insoluble to solvents and has a poor dispersability. Therefore, the surface of a photosensitive member made from the fluorine polymer may be short in lubricity or smoothness, and, having so small a refraction index as to cause light scattering, in transparency. Further, as the fluorine polymer is usually soft, it is susceptible to mechanical damages.

**SUMMARY OF THE INVENTION**

An object of this invention is to provide an electrophotographic photosensitive member to cope with said problems, that is, a photosensitive member free from light scattering and bleeding, being uniform, and having a low surface energy and a high resistance both to mechanical and electrical stresses, a process cartridge inclusive thereof, and an image forming apparatus.

To be more concrete, this invention provides an electrophotographic photosensitive member comprising a substrate and a photosensitive layer thereupon, of which the surface protective layer contains a resin that is produced by curing a curable organosilicon polymer, and an organosilicon-modified positive hole transporting compound represented by the following formula (I):



(where A represents a positive hole transporting group, Q a hydrolyzing group or hydroxyl group, R<sup>2</sup> a substituted or unsubstituted, monovalent hydrocarbon group, R<sup>3</sup> a substituted or unsubstituted alkylene or arylene group, "m" an integer from 1 to 3, and "l" a positive integer).

The present invention also provides a process cartridge and an image forming apparatus, both of which include the electrophotographic photosensitive member.

**BRIEF DESCRIPTION OF THE DRAWINGS**

FIG. 1 is a sectional view of an electrophotographic photosensitive member of this invention to illustrate its layer structure.

FIG. 2 is a sectional view of another electrophotographic photosensitive member of this invention to illustrate its layer structure.

FIG. 3 is a diagram showing the intensity distribution of a spot light, the spot's diameter, the product of the area of the light spot with the thickness of the photosensitive layer, and their relationships.

FIG. 4 is a schematic diagram illustrating the simplified structure of a first example of an image forming apparatus of this invention.

FIG. 5 is a schematic diagram illustrating the simplified structure of a second example of an image forming apparatus of this invention.

FIG. 6 is a H-NMR spectrum of 4-[2-(triethoxysilyl)ethyl]triphenylamine in Synthesis Example 5.

FIG. 7 is a H-NMR spectrum of 4-[N,N-bis(3,4-dimethylphenyl)amino]-[2-(triethoxysilyl)ethyl]benzene in Synthesis Example 8.

FIG. 8 is a C-NMR spectrum of 4-[N,N-bis(3,4-dimethylphenyl)amino]-[2-(triethoxysilyl)ethyl]benzene in Synthesis Example 8.

**DETAILED DESCRIPTION OF THE  
PREFERRED EMBODIMENTS**

The surface layer of the electrophotographic photosensitive member of this invention contains a resin which is produced by curing a curable, organosilicon polymer and an organosilicon-modified hole transporting compound represented by the following formula (I).



(where A represents a hole transporting group, Q a hydrolyzing group or hydroxyl group, R<sup>2</sup> a substituted or unsubstituted, monovalent hydrocarbon group, R<sup>3</sup> a substituted or unsubstituted alkylene or arylene group, m an integer from 1 to 3, and 1 a positive integer).

In the formula (I) Q represents a hydrolyzing group or hydroxyl group, and such hydrolyzing groups may include methoxy group, ethoxy group, methylethylketoxime group, diethylamino group, acetoxy group, propenoxy group, propoxy group, butoxy group, methoxyethyl group, etc., and they should be preferably represented by —OR<sup>1</sup> where R<sup>1</sup> is a group forming alkoxy group or alkoxyalkoxy group which acts as a hydrolyzing group and its carbon number should preferably be an integer between 1 and 6, and may include, for example, methyl group, ethyl group, propyl group, butyl group, pentyl group, hexyl group, methoxyethyl group, etc. Q should preferably be alkoxy group represented by the formula of —OR<sup>1</sup>. Generally speaking, when "m" or the number of the hydrolyzing group bound to the silicon atom is 1, the organosilicon compound itself will not readily undergo condensation, and polymerization will be inhibited. However, when m=2 or 3, the condensation will readily take place, causing highly the cross-linking reaction. Therefore, the compound with m=2 or 3 will give a satisfactory mechanical strength such as the hardness of the resulting cured product, but its highly polymerized product may have an altered solubility, and altered reactivity against silicone thermosetting resins.

R<sup>2</sup> is a monovalent hydrocarbon group directly attached to the silicon atom, and its carbon number should preferably be 1 to 15, and appropriate groups may include, for example, methyl group, ethyl group, propyl group, butyl group, pentyl group, etc. In addition, they may include alkenyl groups such as vinyl group, allyl group, etc., and aryl groups such as phenyl group, tolyl group, etc. The substituent R<sup>2</sup> may contain includes, for example, halogen atoms such as fluorine, and the halogen-substituted monovalent hydrocarbon group includes, for example, fluoro hydrocarbon groups represented by trifluoropropyl group, heptafluoropentyl group, nonafluorohexyl group, etc.

R<sup>3</sup> represents alkylene group or arylene group, and its carbon number should preferably be 1 to 18, and appropriate group may include, for example, methylene group, ethylene group, propylene group, cyclohexylidene group, phenylene group, biphenylene group, naphtylene group, and other groups which are formed by bonding of those groups. The substituent R<sup>3</sup> may contain includes, for example, alkyl groups such as methyl group, ethyl group, etc., aryl groups such as phenyl group, etc., and halogen atoms such as fluorine, chlorine, etc. Of them, R<sup>3</sup> should be preferably represented by the formula —(CH<sub>2</sub>)<sub>n</sub>— where n is a positive integer. Still more preferably n should be an integer between 1 and 18, but the groups may not necessarily have a straight chain form. If "n" is not less than 19 (n≥19), the charge transporting group A will tend to move, and the resulting cured product will tend to have a low hardness. If the charge transporting group is directly bonded to the silicon atom, its steric hindrance will cause impairment of the stability and physical properties of the resulting product. "n" should preferably be 2 to 8, and "l" should preferably be a positive integer between 1 and 5. If "l" is not less than 6 (l≥6), unreacted groups will remain after curing reaction, leading to the impairment of electrical properties.

The charge transporting property mentioned in this invention refers to the ability to transport electric charges, and

should be preferably be 6.2eV or less in terms of ionizing potential. The organosilicon-modified charge transporting compound represented by formula (I) and hydrogen-added A compound should preferably have an ionizing potential of 6.2eV or less, particularly of 4.5 to 6.2eV. If the ionizing potential exceeds 6.2eV, injection of electric charges will become difficult, and the charging will become easy. Conversely, if the ionizing potential is less than 4.5eV, the compound will readily be oxidized, to be subject to deterioration. Ionizing potential can be measured by photoelectron analysis in the atmosphere (Surface Analysis System AC-1, Riken Keiki).

The organosilicon-modified hole transporting compound should preferably have a drift mobility of 1×10<sup>-7</sup> cm<sup>2</sup>/V.sec or more as the hole transporting ability. If it has a drift mobility of less than 1×10<sup>-7</sup> cm<sup>2</sup>/V.sec, is used as an electrographographic photosensitive material, holes will not be able to move sufficiently rapidly in a period between exposure and development, resulting in lowering of apparent sensitivity and leading to elevated residual potential.

The hole transporting group A in the formula (I) given above may be any group capable of transporting holes, and its hydrogen-addition compounds (hole transporting substance) may include, for example, oxazole derivatives, oxadiazole derivatives, imidazole derivatives, triarylamine derivatives such as triphenylamine, 9-(p-diethylaminostyryl)anthracene, 1,1-bis-(4-dibenzylaminophenyl)propane, styrylanthracene, styrylpypyrazoline, phenylhydrazones, α-phenylstyrene derivatives, thiazole derivatives, triazole derivatives, phenazine derivatives, acridine derivatives, benzofuran derivatives, benzimidazole derivatives, thiophene derivatives, N-phenylcarbazole derivatives, etc.

The hole transporting group A should preferably have a structure represented by the following formula (II).



(where R<sup>4</sup>, R<sup>5</sup> and R<sup>6</sup> are organic groups, and at least one of them should be an aromatic hydrocarbon cyclic or heterocyclic group, and R<sup>4</sup>, R<sup>5</sup> and R<sup>6</sup> may be the same, or different each other.)

As is obvious from the above, the hole transporting group A is a group formed by removal of hydrogen atom from one group of R<sup>4</sup>, R<sup>5</sup> and R<sup>6</sup>.

Preferred examples of R<sup>4</sup>, R<sup>5</sup> and R<sup>6</sup> structures will be given below.



—C<sub>p</sub>H<sub>2p+1</sub> p = 1 to 18



5



6



-continued



To synthesize the organosilicon-modified charge transporting compound represented by the above formula (I), a publicly known method, for example, a method whereby a compound having a vinyl group in an aromatic ring and a silicone hydride compound with a substituent are allowed to undergo the hydrosilyl reaction in the presence of a platinum-based catalyst or of an organic peroxide catalyst may be preferably utilized. The platinum catalyst to be used in the method is not limited to any specific ones, but platinum catalysts conventionally used in the hydrosilyl reaction or in the production of addition type silicone rubbers may be profitably used. Thus, appropriate catalysts may include platinum chloride, chloroplatinic acid, platinum-olefin complex, platinum-phosphine complex, etc. No particular limitations are not imposed on the amount of the platinum catalyst, but the amount should be preferably minimized, otherwise the residual catalyst may damage the properties of the compound. When the compound having a vinyl group in an aromatic ring and the silicone hydride compound with a substituent are allowed to undergo the addition reaction in the presence of a platinum-based catalyst or the like to produce a compound of this invention, the reaction may take place at  $\alpha$ - or  $\beta$ -position of the vinyl group. Usually, the resulting compound comprises a mixture of the two isomers. The compound used in this invention may include either of the isomers, but when the hydrocarbon group which binds the charge transporting group to the silicon atom has a lower number of carbon, the isomer formed by the reaction at  $\beta$  position is preferable in terms of the steric hindrance.

The organic peroxide may include any peroxides exhibiting a half life under the environment at room temperature or higher, and particularly alkyl peroxides such as lauryl peroxide may be used preferably because they do not readily extract hydrogens. When a given compound has no vinyl group, formylation is conducted, that is, a formyl group is introduced to the aromatic ring, which is then reduced and dehydrated, or directly subjected to the Wittig reaction, so that the resulting compound may have a vinyl group to be served as a synthetic material for the present invention.

The organosilicon polymer will be explained.

As appropriate silicone polymers can be cited, for example, organopolysiloxane, polysilalkylenesiloxane, polysilarylenesiloxane, etc. Further, the ratio of monovalent hydrocarbon group bonded to the silicon atom against the silicon atoms should preferably be 0.5 to 1.5. As this ratio becomes low with 1.0 as a boundary, the resulting composition may have glass-like composition: the weight loss after heating is reduced, and the resulting composition has an augmented hardness. If the ratio becomes lower than 0.5, the

resulting compound may be hardly able to form a film. Conversely, as the ratio becomes high exceeding 1.0, the tendency in contrast with above emerges. Take organopolysiloxane as an example: when the ratio equals to 2.0, it is converted to polydiorganosiloxane, and when the ratio is more than 1.5, the resulting composition has highly rubber-like properties, and its hardness lowered.

Organopolysiloxane, when used as a material of this invention, should preferably have a structural unit represented by the formula (III):



(where  $R^7$  represents a straight chain or branched alkyl, alkenyl or aryl group,  $R^8$  a hydrogen atom or an alkyl group, and  $r$  and  $s$  molar ratios.)

In the formula (III),  $R^7$  represents a monovalent hydrocarbon group bound to the silicon atom, and should preferably have a carbon number of 1-18. Appropriate straight chain or branched alkyl groups may include, for example, methyl group, ethyl group, propyl group, butyl group, pentyl group, hexyl group, 2-ethylhexyl group, dodecyl group, octadecyl group, etc. Appropriate alkenyl groups may include, for example, vinyl group, allyl group, etc. Appropriate aryl groups may include, for example, phenyl group, tolyl group, etc. Further, halogen-substituted, chain or branched saturated hydrocarbon groups may be mentioned such as fluorohydrocarbon groups represented by trifluoropropyl group, heptafluoropentyl group, nonafluorohexyl group, etc., and chlorohydrocarbon groups such as chloromethyl group, chloroethyl group, etc.,

$R^7$  is not always limited to a specific single kind, but it can exist as a combination of any appropriate groups, according to the target properties of the resin and to the target solubility to a solvent to be used. It has been publicly known that generally, a system comprising methyl and phenyl groups has a stronger affinity to organic compounds than the compound containing methyl group alone. Even organopolysiloxane, when having fluorohydrocarbon group introduced thereto, has, similarly to conventional polymers, a reduced surface tension due to the presence of the fluorine atoms. Therefore, the properties of organopolysiloxane such as water- and oil-repellent activities are changed. In this invention, when the product is desired to have a lower surface tension, silicon units bound to fluorohydrocarbon group can be introduced by the co-polymerization as appropriate.

The molar ratio "r" should preferably be 0.5 to 1.5 on the average.

$OR^8$  group bound to the silicon atom in the formula (III) is a hydroxyl group or a group which can be condensed through hydrolysis.  $R^8$  should be selected from hydrogen or lower alkyl groups comprising methyl group, ethyl group, propyl group, butyl group, etc.  $R^8$  as represented in  $OR^8$  tends to have less reactivity as the carbon number of the alkyl group in question becomes higher starting from hydrogen, and should be appropriately determined according to the reaction system to be used. The fraction of the groups condensable through hydrolysis is represented by the "s" which should preferably be 0.01 or more. It has been publicly known that the hardness of a resin can be controlled through the adjustment of crosslinking density. This can be done also in this invention; the number of the above hydrolysis-condensable groups bound to the silicon atom should be adjusted as appropriate for this purpose. However, if the hydrolysis-condensable group is used too many, unreacted part thereof may remain in the product, and undergo hydrolysis in actual application, thereby impairing the sur-

face property of the final product. The value for "s" should preferably be between 0.01 and 1.5.

One of the characteristics common to organosilicon polymers is their poor affinity to organic compounds or poor solubility to organic compounds. For example, when an oxidation inhibitor or a ultraviolet ray-absorbent commonly used as an additive to the organic resin is introduced into dimethylpolysiloxane, it remains completely undissolved and agglutinates in the resin. Charge transporting compounds commonly used are not an exception to this, and generally they can not be dissolved to a concentration at which they can transport charges smoothly. However, the charge transporting compound of this invention represented by the formula (I) and the organosilicon polymer, particularly organopolysiloxane are well miscible each other, so that the resulting product is greatly improved in its mechanical properties.

The organosilicon polymer may be crosslinked by addition of a cross-linking agent when it is cured.

Further, using a silane compound as represented by formula (IV) below as a cross-linking agent will enable easy control of the physical properties such as hardness and strength of a surface protecting layer obtained by curing a curable composition.



(where  $R^9$  represents a straight chain or branched alkyl, alkenyl, or phenyl group, Y a hydrolyzing group, and "a" a molar ratio.)

In the formula (IV),  $R^9$  should have preferably a carbon number of 1 to 18. It may include, for example, methyl group, ethyl group, propyl group, butyl group, amyl group, hexyl group, vinyl group, allyl group, phenyl group, tolyl group, etc. The hydrolyzing group represented by Y may include hydrogen atom, methoxy group, ethoxy group, methylethylketoxime group, diethylamino group, acetoxy group, propenoxy group, propoxy group, butoxy group, etc.

The above resins do not require necessarily the presence of a catalyst for crosslinking curing, but are compatible with the use of catalysts which have been used for the curing of common organosilicon polymers. When allowance is made for the time and temperature required for curing, alkyltin organic acid salts such as dibutyltin diacetate, dibutyltin dilaurate, dibutyltin octoate, etc. or organic titanate ester such as normal butyl titanate, etc. can be cited as selectable candidates.

Appropriate silane compounds acting as a cross-linking agent and represented by formula (IV) may include, for example, methyltrimethoxysilane, methyltriethoxysilane, vinyltrimethoxysilane, phenyltriethoxysilane, or the above silanes in which the alkoxy groups are substituted by acetoxy group, methylethylketoxime group, diethylamino group, or isopropenoxy group. The cross-linking agent may be an oligomer like ethylpolysilicate.

The method for producing the organosilicon polymer to be used in the present invention includes, in addition to those described in Japanese Patent Publication Nos. 26-2696 and 28-6297, the method for synthesis of organopolysiloxane described in "Chemistry and Technology of Silicones", Chapter 5, p. 191-(Walter Noll, Academic Press, Inc., 1968). For example, organoalkoxysilane or organohalogenosilane in which the number or "r" of monovalent organic groups relative to the silicon atom averages 0.5 to 1.5 is dissolved in an organic solvent, and is hydrolyzed in the presence of an acid or a base such that it polymerizes through condensation. Then, the solvent is removed, and the synthesis is completed. The organosilicon polymer to be employed in

this invention may be used after being dissolved in a solvent chosen from aromatic hydrocarbons such as toluene, xylene, etc., aliphatic hydrocarbons such as cyclohexanone, hexane, etc., halogen hydrocarbons such as chloroform, chlorobenzene, etc., or alcohols such as ethanol, butanol, etc.

In this invention, a curable organosilicon polymer and an organosilicon-modified hole transporting compound take, during curing, a three dimensional structure which prevents the movement among the substituting elements and the entry of chemicals from outside, thereby improving the hardness and mechanical strength of the resulting product, and its resistance to wear. Further, the product can be resistive against electric disturbances such as arc discharges often encountered in association with accumulated electric charges, and against chemical damages.

The solution (also referred to as a curable composition of this invention) containing the above mentioned organosilicon polymer and organosilicon-modified, hole transporting compound before their curing can be obtained, for example, by mixing them in a solvent to which both are soluble. The organosilicon-modified, hole transporting compound should preferably be used in 20 to 200 parts by weight with respect to 100 parts by weight of the solid content of the silicone polymer except for the solvent. If its use amount is less than 20 parts by weight, its hole transporting activity will be reduced, causing increase of the charge potential. If its use amount exceeds 200 weight parts, the resulting product will have a low mechanical strength, and the surface energy will be increased. More preferably 30 to 150 parts by weight of the organosilicon-modified, hole transporting compound should be used with respect to 100 parts by weight of the organosilicon polymer.

In the present invention, parts of a curable polymer and of an organosilicon-modified, hole transporting compound may be allowed to react in advance. In this case, if the resulting solution or dispersant can be applied with no scruples onto a photosensitive member, it will be usable.

Curing should preferably take place by heating at 100° C. to 200° C. If the temperature is 100° C. or lower, the curing reaction takes long, and unreacted hydrolyzing groups may remain after the reaction. If the temperature is 200° C. or higher, the hole transporting group tends to deteriorate through oxidation, thus causing disadvantageous problems. More preferably, curing should take place at 120° C. to 160° C.

An example will be given below to show how a curable composition of this invention capable of transporting holes can be utilized for the manufacture of an electrophotographic photosensitive member.

A substrate (1 in FIGS. 1 and 2) of the electrophotographic photosensitive member can be electroconductive itself and made, for example, of aluminum, aluminum alloys, copper, zinc, stainless steel, chromium, titanium, nickel, magnesium, indium, gold, platinum, silver, iron, etc. Besides, it may be produced after a dielectric substance like plastics has been coated through deposition of aluminum, indium oxide, tin oxide, gold, etc., or it may be produced from a mixture of electroconductive particles with plastics or paper. The electroconductive substrate must have a uniform electroconductivity and a smooth surface. The surface roughness of the substrate should preferably be 0.3  $\mu m$  or less because the smoothness of the surface has great influence on the uniformity of an undercoat layer, a charge generating layer and a charge transporting layer to be formed thereupon. Indentations exceeding 0.3  $\mu m$  greatly affect local electric fields present in thin layers such as the undercoat and charge generating layers, thus altering the proper-

## 11

ties of those layers. Then, injection of charges and residual charges would become uneven.

An electroconductive layer (2 in FIGS. 1 and 2) produced by allowing electroconductive particles to disperse into a polymer binder followed by coating the mixture is easy to form, and can readily give a flat, even surface. The primary particle size of the electroconductive particles used for this purpose should be 100 nm or less, or more preferably 50 nm or less. Appropriate electroconductive particles may include electroconductive zinc oxide, electroconductive titanium oxide, Al, Au, Cu, Ag, Co, Ni, Fe, Carbon black, ITO, tin oxide, indium oxide, indium, etc. These may be coated on the surface of insulating particles. The content of said electroconductive particles should be such that the resulting mixture has a sufficiently low volume resistance, preferably  $1 \times 10^{10} \Omega \cdot \text{cm}$  or less, or more preferably  $1 \times 10^8 \Omega \cdot \text{cm}$  or less.

When a coherent light like laser is used as a source to which the photosensitive member is exposed, said electroconductive substrate can have a rough surface to prevent images formed thereupon from being deteriorated through interference. For this purpose, the surface, to be free from problems such as uneven injection of charges and uneven distribution of residual charges, may be allowed to have indentations about  $\frac{1}{2}\lambda$  or half the wavelength of the incident light, which is achieved after an insulating material like silica beads of less than several  $\mu\text{m}$  in size has been dispersed such that resulting indentations repeat at regular intervals of 10  $\mu\text{m}$  or less.

In the present invention an undercoat layer (3 in FIGS. 1 and 2) capable of intercepting the injection of charges and capable of bonding may be provided between a substrate and a photosensitive layer. The material usable for the undercoat layer may include casein, polyvinylalcohol, nitrocellulose, ethylene-acrylate copolymer, polyvinylbutyral, phenol resins, polyamide, polyurethane, gelatin, etc. The thickness of the undercoat layer should preferably be 0.1 to 10  $\mu\text{m}$ , particularly 0.3 to 3  $\mu\text{m}$ .

A photosensitive layer may have two types: one, or function-separated type comprises a charge generating layer (4 in FIGS. 1 and 2) containing a charge generating material and a charge transporting layer (5 in FIGS. 1 and 2) containing a charge transporting material, and the other, or unity type (not illustrated here) comprises a single layer capable of generating and transporting charges at the same location.

Appropriate charge generating materials may include, for example, selenium-tellurium and pyryliumbased dye, thiopyrylium-based dye, phthalocyanine-based pigment, anthanthrone-based pigment, dibenzpyrenequinone-based pigment, pyranthrone-based pigment, trisazo-based pigment, disazo-based pigment, azo-based pigment, indigo-based pigment, quinacrydone-based pigment, cyanin-based pigment, etc.

A cured product produced from a curable composition of this invention capable of transporting holes can be used for a charge transporting layer (5 in FIG. 1) or for a surface-protecting layer (6 in FIG. 2) capable of transporting holes.

In case of a unity type of photosensitive member, the charge generating substance and the curable composition of this invention capable of transporting holes may be combined so that good properties can be obtained.

The curable composition of this invention capable of transporting holes can be used in combination with other charge transporting substances. Such charge transporting substances may include high molecular transporting substances may include high molecular compounds polymers with a heterocycle or condensed polycyclic aromatic such as

## 12

poly-N-vinylcarbazole, polystyrylanthracene, etc., and low molecular compounds such as heterocyclic compounds like pyrazoline, imidazole, oxazole, oxadiazole, triazole, carbazole, etc., triarylalkane derivatives like triphenylmethane, phenylenediamine derivatives, N-phenylcarbazole derivatives, styrene derivatives, hydrazone derivatives, etc.

The charge generating substance or charge transporting substance may be supplemented as appropriate with a binder polymer. Appropriate binder polymers may include, for example, polymers or copolymers of vinyl compounds such as styrene, vinyl acetate, vinyl chloride, acrylate ester, methacrylate ester, vinylidene fluoride, trifluoroethylene, and polyvinyl alcohol, polyvinyl acetal, polycarbonate, polyester, polysulfone, polyphenylene oxide, polyurethane, cellulose resins, phenol resins, melamine resins, silicone resins, epoxy resins, etc.

A curable composition of this invention capable of transporting holes may be supplemented with other additives, in addition to above compounds, to improve mechanical properties or durability of the product. Such additives may include oxidation inhibitors, ultra-violet ray absorbents, stabilizers, lubricants, electroconductivity adjusters, etc.

The thickness of the charge generating layer of this invention should preferably be 3  $\mu\text{m}$  or less, particularly 0.01 to 1  $\mu\text{m}$ . The thickness of the charge transporting layer should preferably be 1 to 40  $\mu\text{m}$ , particularly 3 to 30  $\mu\text{m}$ . When the photosensitive layer is of unity, or monolayer type, its thickness should preferably be 1 to 40  $\mu\text{m}$ , particularly 3 to 30  $\mu\text{m}$ .

The thickness of a surface protecting layer of this invention should preferably be 1 to 15  $\mu\text{m}$ . If it is 1  $\mu\text{m}$  or less, the protection will not be satisfactory. If it exceeds 15  $\mu\text{m}$ , it will add to the overall thickness of the photosensitive layer, thereby causing deterioration in the quality of images.

In the present invention, the product of a spot area an exposure means forms on the photosensitive surface and the thickness or depth of the photosensitive layer within the photosensitive member should preferably be  $2 \times 10^4 \mu\text{m}^3$  or less. Further, this product should be  $2 \times 10^3 \mu\text{m}^3$  or more in terms of the development contrast (potential difference on the photosensitive member during developing). If the product is less than  $2 \times 10^3 \mu\text{m}^3$ , sufficient contrast will not be obtained during developing.

In this case, light exposure used in this invention consists of directing light in the form of dots onto a photosensitive member to produce electrostatic latent images there. The light source is not limited to any specific one, but should preferably be a laser or an LED light because they allow easy production of a small light spot area.

FIG. 3 gives the intensity distribution of a spot light, the spot's diameter, the product of the area (S) of the light spot with the thickness of the photosensitive layer, and their relationships. The light spot generally has a shape of ellipse comprising a diameter (ab) in the main scanning direction and another diameter (cd) in the subsidiary scanning direction. The product of the area of the light spot and the thickness of the photosensitive layer of this invention represents, so to say, the volume (V) of the photosensitive layer exposed to the light.

The spot area (S) formed by the light represents an area on the photosensitive layer exposed to the light, and corresponds to the area at which the incident light has an intensity of  $1/e^2$  (B) of the peak intensity (A), or more. The usable light source may include a semiconductor laser, LED, etc., and the light intensity can take a Gaussian distribution or a Lorenz distribution. In any case, the spot area (S) is defined

## 13

by the area at which incident light has an intensity of  $1/e^2$  (B) of the peak intensity (A), or more. The spot area (S) can be measured by using a CCD camera which is put in place of the photosensitive member.

In this invention, the spot area should preferably be  $4 \times 10^3 \mu\text{m}^2$  or less, particularly  $3 \times 10^3 \mu\text{m}^2$  or less. If it exceeds  $4 \times 10^3 \mu\text{m}^2$ , spots of adjacent pixels tend to merge, thus hampering tone reproducibility. The spot area of  $1 \times 10^3 \mu\text{m}^2$  or more will be beneficial also in terms of cost.

From above considerations, a photosensitive layer of this invention should preferably have a thickness of  $12 \mu\text{m}$  or less, particularly  $10 \mu\text{m}$  or less.

An electrophotographic photosensitive member of this invention has an excellent mechanical strength and a good surface lubricity, and is well adapted to be used for above lighting systems.

FIG. 4 gives a schematic diagram illustrating the simplified structure of a first example of an image forming apparatus having a process cartridge of this invention.

In the figure, 7 is a drum-shaped electro-photographic photosensitive member of this invention, and is driven into rotation around an axis 8 at a predetermined circumferential speed in the direction the arrow indicates. The photosensitive member 7 receives, during rotation, upon its circumference an even distribution of positive or negative charges having a predetermined potential from a charging means 9. Then, it receives an imagewise exposure light 10 emitted from an imagewise exposure means (not illustrated here) such as laser beam-scanning exposure means, etc. Thus, electrostatic latent images are formed successively on the circumferential surface of the photosensitive member 7.

The electrostatic latent images thus formed are developed with a toner using a developing means 11, and the toner images thus developed are transferred successively by a transferring means 12 to a transfer material 13 which is fed, in synchrony with the rotation of the photosensitive member 7, into between the photosensitive member 7 and a transferring means 12 from a paper feeding section (not illustrated here).

The transfer material 13 having images transferred thereupon is separated from the photosensitive member, and is introduced into a image-fixing means 14 to have the image fixed thereby. The images thus printed on the sheet are discharged from the system as a print-out.

The photosensitive member 7 has its surface cleaned, after transferring of the image, by a cleaning means 15. Thus, the surface is removed of residual toners to be kept clean, and then is removed of residual charges by receiving a priming light 16 from a pre-exposure means (not illustrated here) to be ready for further use to form images. If a primary charging means 9 works through direct contact, for example, by the use of a charging roller, the priming light is not always necessary.

In the present invention, a plurality of such constituent elements as said electrophotographic photosensitive member 7, primary charging means 9, developing means 11 and cleaning means 15 may be united to be installed into a housing to serve as a process cartridge which can be reversibly mounted to an image forming system such as a copying machine, a laser-beam printer, etc. For example, at least one from the primary charging means 9, developing means 11 and cleaning means 15 may be combined with the photosensitive member 7 into a process cartridge 17, which, then, may be reversibly mounted to a main system by sliding on a pair of rails 18 prepared therein.

FIG. 5 gives a schematic diagram illustrating the simplified structure of a second example of an image forming apparatus of this invention, or a color copying machine.

## 14

In the figure, numeral 201 represents an image scanner section which reads a manuscript and translates it into digital signals. Numeral 202 is a printer section which prints, onto a sheet of paper, an image in full color corresponding to the original image read by the image scanner 201.

With regard to the image scanner section 201, 200 is a mirror-faced thick plate, a manuscript 204 is placed on a manuscript glass plate 203, and the manuscript is exposed to light which has been generated by a halogen lamp 205 and allowed to pass through a filter 208 intercepting infra-red lights. The light reflected from the manuscript is guided to mirrors 206 and 207, and through a mirror 209 to be focused onto a 3 line sensor (CCD) 210. The full color information comprising red (R), green (G) and blue (B) components is sent to a signal processing section 211. 205 and 206 are mechanically driven at a velocity of  $v$ , and 207 at a velocity of  $1/2 v$  in the direction vertical (in the subsidiary scanning direction) to the direction (main scanning direction) towards which the line sensor is driven electrically, thereby scanning the whole surface of the manuscript.

The signal processing section 211 electrically processes signals read from the manuscript, decomposes them into individual components such as magenta (M), cyan (C), yellow (Y) and black (BK), which are then transferred to a printer section 202. Each time one whole surface of a manuscript is scanned by the image scanner section 201, one of M, C, Y and BK is sent to the printer 202: thus whenever a manuscript is scanned four times in succession, one printout is dispatched.

M, C, Y and BK image signals delivered by the image scanner section 201 are carried to a laser driver 212 which modulates a semiconductor laser generator 213 according to the image signals. Laser light, passing through a polygon mirror 214, an f-θ lens 215 and a mirror 216, scans the surface of a photosensitive member 217.

218 is a rotatory developer and comprises a magenta developer 219, a cyan developer 220, a yellow developer 221, and a black developer 222 in such a way that the four developers come into contact with the photosensitive member in succession, and develop M, C, Y and BK electrostatic latent images which are formed on the photosensitive member 217 with the corresponding toners.

Numerical 223 denotes a transferring drum, round which a sheet of paper fed from a paper cassette 224 or 225 is wound, and whereby the toner image developed on the photosensitive member 217 is transferred onto the sheet of paper.

Through such mechanism, four colors represented by M, C, Y and BK are transferred in succession onto the sheet of paper which then is passed through a fixing unit 226 to be discharged from the system.

Then, examples will be given to illustrate how the curable organosilicon polymer of this invention can be synthesized.

## Synthesis Example 1

Preparation of solution of cure type resin chiefly composed of methylpolysiloxane resin:

In 10 g of toluene, was dissolved 10 g of methylpolysiloxane resin containing 1% by weight of silanol group and comprised of 80 mol % of methylsiloxane unit and 20 mol % of dimethylsiloxane unit. To the resulting solution, 5.3 g of methyltrimethoxysilane and 0.2 g of dibutyltin diacetate were added to make a uniform solution.

## Synthesis Example 2

Preparation of solution of cure type resin chiefly composed of methylpolysiloxane resin:



Thereafter, the precipitate formed was collected by filtration, and washed with a mixture of ethanol/water (1:1) to obtain tri-(4-formylphenyl)amine in an amount of 65.3 g (yield: 95.9%).

#### Synthesis of tri(4-vinylphenyl)amine

Into a three-necked flask, 14.6 g of sodium hydride and 70 ml of 1,2-dimethoxyethane were placed, and 130.8 g of trimethylphosphonium bromide was added thereto with stirring at room temperature. Next, after a drop of absolute alcohol was added, the reaction was allowed to proceed at 70° C. for 4 hours. Then, 40.2 g of tri(4-formylphenyl)amine was added to the mixture thus obtained, to carry out reaction at 70° C. for 5 hours. The reaction solution obtained was filtered to remove the cake. The ether extract of the cake was put together with the filtrate, and washed with water. Then, the ether solution was dehydrated with calcium chloride, and thereafter ether was removed to obtain a reaction mixture. After twice recrystallization with ethanol, accusal pale yellow tri(4-vinylphenyl)amine was obtained in an amount of 38.4 g (yield: 97.3%).

#### Hydrosilylation of tri(4-vinylphenyl)amine

Into a three-necked flask, 40 ml of toluene, 9.9 g (60 mmol) of triethoxysilane and 0.018 mmol of diplatinum (0) tris(tetramethyldivinyldisiloxane) in toluene were placed, and 20 ml of a toluene solution containing 3.3 g (13 mmol) of tri(4-vinylphenyl)amine was added dropwise with stirring at room temperature. After the addition was completed, the mixture was stirred at 70° C. for 3 hours, and thereafter the solvent was removed under reduced pressure to obtain oily pale yellow 4,4',4"-tris[2-(triethoxysilyl)ethyl]triphenylamine in an amount of 7.8 g (yield: 80.6%).

Ionization potential of this compound measured by atmospheric photoelectron analysis (using a surface analyzer AC-1, manufactured by Riken Keiki K.K.) was 5.65 eV.

This compound was applied onto a substrate of copper by the wirebar coat method and subjected to thermal curing treatment at 120° C. for 12 hours to form a film of about 5  $\mu$ m. Next, a semi-transparent electrode of gold was formed by the vapor deposition.

The drift mobility of this sample was measured by the Time-of-flight method using a nitrogen laser with a pulse width of 3 nsec. End a wavelength of 337 nm and found to be  $3 \times 10^{-7} \text{ cm}^2/\text{Vsec}$ .

#### Synthesis Example 8

##### Synthesis of 4-[N,N-bis(3,4-dimethylphenyl)amino]-[2-(triethoxysilyl)ethyl]benzene

##### Synthesis of N,N-bis(3,4-dimethylphenyl)aminobenzene

To 20 ml of nitrobenzene, 38.5 g (166 mmol) of 4-iodo-o-xylene, 22.9 g (166 mmol) of anhydrous potassium carbonate and 7.0 g of copper powder were added, followed by heating and reflux for 8 hours with stirring. The reaction mixture was cooled and filtered, and the precipitate was removed. The filtrate (crude reaction product) was passed through a silica gel column to obtain 15.7 g of N,N-bis(3,4-dimethylphenyl)aminobenzene (yield: 69%).

##### Synthesis of 4-[N,N-bis(3,4-dimethylphenyl)amino]benzaldehyde

Into a three-necked flask, 124.6 g of [N,N-bis(3,4-dimethylphenyl)amino]benzene and 35.5 ml of DMF were placed, and 84.4 ml of phosphorus oxychloride was added

dropwise thereto with stirring while cooling with ice water. After the addition was completed, the mixture solution was heated to 95° C. to carry out reaction for 5 hours. The reaction solution obtained was poured into 4 liters of warm water, followed by stirring for 1 hour. Thereafter, the precipitate was collected by filtration, and washed with a mixture of ethanol/water (1:1) to obtain 4-[N,N-bis(3,4-dimethylphenyl)amino]benzaldehyde in an amount of 107.6 g (yield: 79.0%).

##### Synthesis of 4-[N,N-bis(3,4-dimethylphenyl)amino]styrene

Into a three-necked flask, 12.1 g of sodium hydride and 580 ml of 1,2-dimethoxyethane were placed, and 108.5 g of trimethylphosphonium bromide was added thereto with stirring at room temperature. Next, after a drop of absolute alcohol was added, the reaction was allowed to proceed at 70° C. for 4 hours. Then, 100.0 g of 4-[N,N-bis(3,4-dimethylphenyl)amino]benzaldehyde was added to the reaction mixture, to carry out reaction at 70° C. for 5 hours, followed by filtration to collect a cake. The cake was extracted with ether and the extract was put together with the filtrate and washed with water. Then, the ether solution was dehydrated with calcium chloride, and thereafter the ether was removed to obtain a crude product. After twice recrystallized from ethanol, accusal 4-[N,N-bis(3,4-dimethylphenyl)amino]styrene was obtained in an amount of 84.5 g (yield: 85.0%).

##### Hydrosilylation of 4-[N,N-bis(3,4-dimethylphenyl)amino]styrene

Into a three-necked flask, 40 ml of toluene, 6.0 g of triethoxysilane and 0.54 mmol of diplatinum (0) tris(tetramethyldivinyldisiloxane) in toluene were placed, and 20 ml of a toluene solution containing 9.9 g of 4-[N,N-bis(3,4-dimethylphenyl)amino]styrene was added dropwise with stirring at room temperature. After the addition was completed, the mixture was stirred at 70° C. for 3 hours, and thereafter the solvent was removed under reduced pressure to obtain oily pale yellow 4-[N,N-bis(3,4-dimethylphenyl)amino]-[2-(triethoxysilyl)ethyl]benzene in an amount of 13.4 g (yield: 90.1%).

An H-NMR spectrum (measured by APC300, an NMR spectrometer manufactured by Bruker Co.) of the compound obtained is shown in FIG. 7. A C-NMR spectrum (measured by APC300, an NMR spectrometer manufactured by Bruker Co.) of the product compound is shown in FIG. 8.

Ionization potential of this compound measured by atmospheric photoelectron analysis (using a surface analyzer AC-1, manufactured by Riken Keiki K.K.) was 5.26 eV.

This compound was applied onto a substrate of copper by the wirebar coat method and subjected to thermal curing treatment at 120° C. for 12 hours to form a film of about 5  $\mu$ m. Next, a semi-transparent electrode of gold was formed by the vapor deposition.

The drift mobility of this sample was measured by the Time-of-flight method using a nitrogen laser with a pulse width of 3 nsec. End a wavelength of 337 nm and found to be  $9 \times 10^{-7} \text{ cm}^2/\text{Vsec}$ .

#### Synthesis Example 9

##### Synthesis of 4-[N,N-bis(3,4-dimethylphenyl)amino]-[2-(triethoxysilyl)ethyl]benzene

##### Hydrosilylation of 4-[N,N-bis(3,4-dimethylphenyl)amino]styrene

Into a three-necked flask, 40 ml of toluene, 6.0 g (37 mmol) of triethoxysilane and 0.34 mmol of platinum (II)

## 19

dichloro(h-cycloocta-1,5-diene) were placed, and 20 ml of a toluene solution containing 9.9 g of 4-[N,N-bis(3,4-dimethylphenyl)amino]styrene was added dropwise with stirring at room temperature. After the addition was completed, the mixture was stirred at 70° C. for 3 hours, and thereafter the solvent was removed under reduced pressure to obtain oily pale yellow 4-[N,N-bis(3,4-dimethylphenyl)amino]-[2(triethoxysilyl)ethyl]benzene in an amount of 14.0 g (yield: 94.2%).

Ionization potential of this compound measured by atmospheric photoelectron analysis (using a surface analyzer AC-1, manufactured by Riken Keiki K.K.) was 5.31 eV. thermal curing treatment at 120° C. for 12 hours to form a film of about 5  $\mu$ m. Next, a semi-transparent electrode of gold was formed by the vapor deposition.

The drift mobility of this sample was measured by the Time-of-flight method using a nitrogen laser with a pulse width of 3 nsec. End a wavelength of 337 nm and found to be  $7 \times 10^{-7} \text{ cm}^2/\text{Vsec}$ .

## Synthesis Example 10

## Synthesis of 4-[3-(triethoxysilyl)propyl] triphenylamine

## Synthesis of 4-bromotriphenylamine

Into a 200 ml three-necked flask, 8.0 g (45 mmol) of N-bromosuccinimide and 10.0 g (41 mmol) of triphenylamine were placed, followed by 150 ml of N,N-dimethylformamide. The mixture was stirred overnight at room temperature. Next, N,N-dimethylformamide was removed from the reaction, and the resulting solid matter was extracted with carbon tetrachloride. Then, carbon tetrachloride was removed, and the reaction product was recrystallized twice from ethanol to give a white solid, 4-bromotriphenylamine in an amount of 8.2 g (yield: 61.7%).

## Synthesis of 4-N,N-diphenylaminoallylbenzene

Into a 300 ml four-necked flask, 1.0 g (40 mmol) of magnesium metal was placed, and the space air was replaced with nitrogen. Subsequently, 100 ml of

Into a 300 ml four-necked flask, 1.0 g (40 mmol) of magnesium metal was placed, and the space air was replaced with nitrogen. Subsequently, 100 ml of diethyl ether was added and stirring was started. To the mixture being stirred, 30 ml of diethyl ether solution dissolving 8.6 g (27 mmol) of 4-bromotriphenylamine was slowly added dropwise. When about 3 ml of the 4-bromotriphenylamine solution was added dropwise, reflux slowly began. While being refluxed, the remaining 4-bromotriphenylamine solution was added dropwise. After the addition was completed, the reflux was further continued for 1 hour to obtain a Grignard reagent solution. The reagent solution thus obtained was cooled to room temperature, and then 40 ml of a diethyl ether solution containing 2.1 g (27 mmol) of allyl chloride was slowly added dropwise while cooling with ice. After the addition was completed, the reaction mixture was refluxed for 2 hours to age the reaction. Thereafter, 50 ml of water was added while cooling with ice, to effect hydrolysis. Next, the ether layer was collected, washed once with a saturated aqueous sodium hydrogencarbonate solution and washed twice with water, and then dried with anhydrous sodium sulfate. After drying, diethyl ether was removed to obtain a white solid, 4-N,N-diphenylaminoallylbenzene in an amount of 4.9 g (yield: 63.2%).

## 20

## Hydrosilylation of 4-N,N-diphenylaminoallylbenzene

Into a three-necked flask, 40 ml of toluene, 6.0 g (37 mmol) of triethoxysilane and 0.54 mmol of diplatinum (0) tris(tetramethyldivinyldisiloxane) in toluene were placed, and 20 ml of a toluene solution containing 9.7 g (34 mmol) of 4-N,N-diphenylaminoallylbenzene was added dropwise with stirring at room temperature. After the addition was completed, the mixture was stirred at 70° C. for 3 hours, and thereafter the solvent was removed under reduced pressure to obtain oily pale yellow 4-[3-(triethoxysilyl)propyl] triphenylamine in an amount of 10.7 g (yield: 70.1%).

Ionization potential of this compound measured by atmospheric photoelectron analysis (using a surface analyzer AC-1, manufactured by Riken Keiki K.K.) was 5.72 eV.

This compound was applied onto a substrate of copper by the wirebar coat method and subjected to thermal curing treatment at 120° C. for 12 hours to form a film of about 9  $\mu$ m. Next, a semi-transparent electrode of gold was formed by the vapor deposition.

The drift mobility of this sample was measured by the Time-of-flight method using a nitrogen laser with a pulse width of 3 nsec. End a wavelength of 337 nm and found to be  $1.4 \times 10^{-7} \text{ cm}^2/\text{Vsec}$ .

## Synthesis Example 11

## Synthesis of 4-[4-(triethoxysilyl)butyl] triphenylamine

## Synthesis of 4-methyltriphenylamine

To 30 ml of o-dichlorobenzene, 4.5 g (27 mmol) of diphenylamine, 11.0 g (51 mmol) of p-iodotoluene, 5.5 g (40 mmol) of anhydrous sodium carbonate and 1.1 g of copper powder were added. The mixture was heated and refluxed with stirring for 7 hours. After the reaction was completed, the reaction solution was filtered. The filtrate was successively washed with an aqueous 35% sodium thiosulfate solution and saturated brine. The organic layer was dried with anhydrous sodium sulfate, and thereafter the solvent was removed. The resulting crude reaction product was recrystallized from ethanol to obtain 4-methyltriphenylamine in an amount of 5.7 g (yield: 81.4%).

## Synthesis of 4-bromomethyltriphenylamine

Into a 300 ml three-necked flask, 6.9 g (39 mmol) of N-bromosuccinimide and 9.1 g (35 mmol) of 4-methyltriphenylamine were placed, and 100 ml of carbon tetrachloride was added thereto. Thereafter, the mixture was heated and refluxed overnight with stirring. After the reaction was completed, the reaction solution was cooled. Subsequently, the reaction was filtered, and the solvent was removed. The reaction product thus obtained was recrystallized from ethanol to obtain 4-bromomethyltriphenylamine in an amount of 10.8 g (yield: 91.2%).

## Synthesis of 4-N,N-diphenylaminophenyl-1-butene

Into a 200 ml four-necked flask, 1.0 g (40 mmol) of magnesium metal was put, and the space air of the flask was replaced with nitrogen. Subsequently, 100 ml of diethyl ether was added and stirring was started. To the mixture, 20 ml of a diethyl ether solution in which 9.1 g (27 mmol) of 4-bromomethyltriphenylamine was dissolved was slowly added dropwise with stirring. When about 5 ml of the

21

solution was added dropwise, reflux slowly started. While being refluxed, the remaining solution of 4-bromomethyltriphenylamine was added dropwise. After the addition was completed, the reflux was further continued for 1 hour to obtain a Grignard reagent solution. The reagent solution thus obtained was cooled to room temperature, and then 20 ml of a diethyl ether solution of 2.1 g (27 mmol) of allyl chloride was slowly added dropwise while cooling with ice. After the addition was completed, the reaction mixture was refluxed for 2 hours to age the reaction. Thereafter, 50 ml of water was added while cooling with ice, to effect hydrolysis. Next, the ether layer formed was collected, washed once with a saturated aqueous sodium hydrogencarbonate solution and twice with water, and then dried with anhydrous sodium sulfate. After drying, diethyl ether was removed to obtain a white solid, 4-N,N-diphenylaminophenyl-1-butene in an amount of 5.5 g (yield: 66.7%).

Hydrosilylation of 4-N,N-diphenylaminophenyl-1-butene

Into a three-necked flask, 40 ml of toluene, 9.9 g (60 mmol) of triethoxysilane and 0.018 mmol of diplatinum (0) tris(tetramethyldivinyldisiloxane) in toluene were placed, and 20 ml of a toluene solution containing 16.7 g (54.7 mmol) of 4-N,N-diphenylaminophenyl-1-butene was added dropwise with stirring at room temperature. After the addition was completed, the mixture was stirred at 70° C. for 3 hours, and thereafter the solvent was removed under reduced pressure to obtain oily pale yellow 4-[4-(triethoxysilyl)butyl]triphenylamine in an amount of 13.9 g (yield: 83.2%).

Ionization potential of this compound measured by atmospheric photoelectron analysis (using a surface analyzer AC-1, manufactured by Riken Keiki K.K.) was 5.69 eV.

This compound was applied onto a substrate of copper by the wirebar coat method and subjected to thermal curing treatment at 120° C. for 12 hours to form a film of about 5  $\mu\text{m}$ . Next, a semi-transparent electrode of gold was formed by the vapor deposition.

The drift mobility of this sample was measured by the Time-of-flight method using a nitrogen laser with a pulse width of 3 nsec. and a wavelength of 337 nm and found to be  $2 \times 10^{-7} \text{ cm}^2/\text{Vsec.}$

Synthesis Example 12

In the resin solution of Synthesis Example 1, 4-[2-(triethoxysilyl)ethyl]triphenylamine (Synthesis Example 5) was added in an amount of 70% by weight based on the weight of the resin solid matter and mixed. The mixture was applied on a glass plate by means of a bar coater, followed by drying at 140° C. for 15 hours. Under microscopic observation, a uniform film had been formed.

Comparative Synthesis Example 1

In the resin solution of Synthesis Example 1, triphenylamine was dissolved as a charge transporting compound in an amount of 30% by weight based on the weight of the resin, followed by mixing and curing in the same manner as in Synthesis Example 12 to form a film. The film was cloudy, and microscopic observation confirmed deposition of triphenylamine.

Comparative Synthesis Example 2

The procedure of Comparative Synthesis Example 1 was repeated to form a film, except that the resin solution of

22

Synthesis Example 2 was used. The film formed was less opaque, but microscopic observation confirmed deposition of crystals of triphenylamine.

Comparative Synthesis Example 3

The procedure of Synthesis Example 6 was repeated to obtain 4-[2-(trimethylsilyl)ethyl]triphenylamine, except that 6 g (60 mmol) of trimethylsilane was used in the hydrosilylation of the 4-vinyltriphenylamine obtained in Synthesis Example 5. Using this, a film was formed in the same manner as in Comparative Example 1. As a result, the film was opaque, and separation of 4-[2-(trimethylsilyl)ethyl]triphenylamine was observed.

Synthesis Example 13

Synthesis of 4-(N-ethyl-N-phenylamino)-[2-(triethoxysilyl)ethyl]benzene

Synthesis of 4-(N-ethyl-N-phenylamino)-benzaldehyde

Into a three-necked flask, 82 g of diphenylethylamine and 35.5 ml of DMF were added, and 84.4 ml of phosphorus oxychloride was added dropwise thereto with stirring while cooling with ice water. After the addition was completed, the temperature was raised to 95° C. to carry out reaction for 5 hours. Thereafter, the resulting precipitate was collected by filtration, and washed with a mixture of ethanol/water (1:1) to obtain 4-(N-phenylamino)benzaldehyde in an amount of 62 g.

Synthesis of 4-(N-ethyl-N-phenylamino)styrene

Into a three-necked flask, 14.6 g of sodium hydride and 700 ml of 1,2-dimethoxyethane were placed, and 130.8 g of trimethylphosphonium bromide was added thereto with stirring at room temperature. Next, after a drop of absolute alcohol was added, the reaction was allowed to proceed at 70° C. for 5 hours. The reaction solution was filtered, and the filtrate and an ether-extract of the precipitate were put together, followed by washing with water. Then, the ether fraction was dehydrated with calcium chloride, and thereafter the ether was removed to obtain a crude reaction product. The reaction product was recrystallized from ethanol to obtain acicular pale yellow crystals in an amount of 62.4 g.

Hydrosilylation of 4-(N-ethyl-N-phenylamino)-styrene

Into a three-necked flask, 40 ml of toluene, 9.9 g (60 mmol) of triethoxysilane and 0.018 mmol of diplatinum (0) tris(tetramethyldivinyldisiloxane) in toluene were placed, and 20 ml of a toluene solution containing 7.6 g of 4-(N-ethyl-N-phenylamino)styrene was added dropwise with stirring at room temperature. After the addition was completed, the mixture was stirred at 70° C. for 3 hours, and then the solvent was removed under reduced pressure to obtain oily pale yellow 4-(N-ethyl-N-phenylamino)-[2-(triethoxysilyl)ethyl]benzene in an amount of 7.8 g.

Ionization potential of this compound measured by atmospheric photoelectron analysis (using a surface analyzer AC-1, manufactured by Riken Keiki K.K.) was 6.3 eV.

This compound was applied onto a substrate of copper by the wirebar coat method and subjected to thermal curing treatment at 120° C. for 12 hours to form a film of about 5  $\mu\text{m}$ . Next, a semi-transparent electrode of gold was formed by the vapor deposition.

23

The drift mobility of this sample was measured by the Time-of-flight method using a nitrogen laser with a pulse width of 3 nsec and a wavelength of 337 nm and found to be  $2 \times 10^{-8} \text{ cm}^2/\text{Vsec}$ .

## EXAMPLE 1

A solution produced by dissolving 5 parts by weight of alcohol soluble copolymer nylon (tradename: Amilan CM-8000, Toray) into 95 parts by weight of methanol was applied through immersion coating onto the outer surface of an aluminum cylinder with an outer diameter of 80 mm which had undergone surface processing. It was allowed to dry at 80° C. for 10 min to produce a 1  $\mu\text{m}$  thick undercoat layer.

Then, 5 parts by weight of a bisazo pigment described below were added to a solution which was produced by dissolving 2 parts by weight of polyvinylbenzal (benzal conversion being 75% or more) into 95 parts by weight of cyclohexanone, and the mixture was dispersed with a sand-mill to prepare a dispersant for a charge generating layer.

The resulting dispersant was applied through immersion coating onto the undercoat layer in such a manner that the resulting layer, after being dried, had a thickness of 0.2  $\mu\text{m}$ .



Then, to a solution produced by dissolving 5 parts by weight of triarylamine compound having a structure described below and 5 parts by weight of a polycarbonate resin (tradename: Z-200, Mitsubishi Gas Chemical) in 70 parts by weight of chlorobenzene, which solution serves as a material of an electric charge transporting layer, added was 0.3 part by weight of silicone resin fine particles having an average particle diameter of 2  $\mu\text{m}$ , and the mixture was applied through immersion coating onto the above charge generating layer in such a manner that the newly added layer, after being dried, had a thickness of 10  $\mu\text{m}$ .



Then, a curable composition produced by adding 200 parts by weight of toluene and 40 parts by weight of 4-[N,N-bis(3,4-dimethylphenyl)amino]-[2-(triethoxysilyl)ethyl]benzene synthesized in Synthesis Example 8 to 100

24

parts by weight of the curable composition synthesized in Synthesis Example 1 was applied through spray coating.

The assembly was allowed to dry at 140° C. for 4 hours, and a transparent, even surface-protecting layer with a thickness of 2  $\mu\text{m}$  was formed thereupon through thermal curing.

The resulting electrophotographic photosensitive member, after being charged with -700V, was exposed to light with a wavelength of 680 nm, and its photographic performance was studied: E1/2 (light exposure necessary for lowering the charge to -350V) was 1.2  $\mu\text{J}/\text{cm}^2$  and the residual potential was -26V. The performance was satisfactory.

A Canon-manufactured digital full-color copying machine (CLC-500) was so modified as to give a spot having a diameter ( $1/e^2$ ) of 63.5  $\mu\text{m}$  in the subsidiary scanning direction, and of 20  $\mu\text{m}$  in the main scanning direction, to test the photosensitive member of this Example. The initial charging potential was set to -500V and the electrophotographic performance of the photosensitive member was studied. The photosensitive member gave satisfactory results: the images showed no black dots due to stray injection of charges and no interference streaks even after a 100,000 sheet continuous running test as well as at the initial

stage of the test; the wear of the photosensitive member after the test was only 0.8  $\mu\text{m}$ ; it gave images excellent in uniformity; and its tone reproducibility was also good, giving 256 tones at 400 dpi.

## Comparative Synthesis Example 4

Into 100 parts by weight of the resin solution in Synthesis Example 4 was dissolved the triarylamine compound used in Example 1 in an amount of 30 weight % with respect to the amount of the resin, and the mixture was treated and cured in the same manner as in Synthesis Example 12 to produce a film. The film had white turbidity, and, when observed under microscope, showed deposition of triphenylamine.

## Comparative Example 1

An electrophotographic photosensitive member produced in the same manner as in Example 1 except that no protective layer was coated evaluated of its electrophotographic performance. After it had undergone a 20,000 sheet running test, it suffered a great number of black dots and the quality of images thereupon was impaired. The wear of the photosensitive member was as large as 5  $\mu\text{m}$  after 20,000 sheets.

## EXAMPLE 2

167 Parts by weight of a phenol resin (tradename: Plyophen, Dainippon Ink & Chemicals) were dissolved into

## 25

100 parts by weight of methylcellosolve, to which were added 200 parts by weight of electroconductive barium sulfate ultra-fine particles (primary particle size being 50 nm) and 3 parts by weight of silicone resin particles having an average diameter of 2  $\mu\text{m}$ . The mixture, after being dispersed, was applied through immersion coating onto the outer surface of an aluminum cylinder with an outer diameter of 30 mm which had been prepared through extraction processing. The coat was dried to produce a 15  $\mu\text{m}$  thick electroconductive layer.

A solution produced by dissolving 5 parts by weight of alcohol soluble copolymer nylon (tradename: Amilan CM-8000, Toray) into 95 parts by weight of methanol was applied through immersion coating onto above electroconductive layer. The coat was allowed to dry at 80° C. for 10 min to produce a 1  $\mu\text{m}$  thick undercoat layer.

Then, 5 parts by weight of an oxytitaniumphthalocyanine pigment which has high peaks at Bragg angles ( $20\pm0.2$ ) of 9.0°, 14.2°, 23.9° and 27.1° when examined by CuK $\alpha$  characteristic X-ray analysis, was added to a solution which was produced by dissolving 2 parts by weight of polyvinylbenzal (benzal conversion being 75% or more) into 95 parts by weight of cyclohexanone, and the mixture was dispersed with a sandmill to prepare a dispersant of the charge generating layer.

The resulting dispersant was applied through immersion coating onto the undercoat layer in such a manner that the resulting layer, after being dried, had a thickness of 0.2  $\mu\text{m}$ .

Then, 55 parts by weight of organosilicon-modified triarylamine compound synthesized in Synthesis Example 9 and 100 parts by weight of silicone thermosetting resin in Synthesis Example 3 were added to 100 parts by weight of toluene for dissolution. The mixture was applied through immersion coating onto the charge generating layer. It was dried at 120° C. for 5 hours for thermal curing, to form a clear, uniform charge transporting layer of 10  $\mu\text{m}$  thickness.

Its pencil hardness was 5H, and has an angle of 105° in contact with water.

The resulting electrophotographic photosensitive member, after being charged with -700V, was exposed to light with a wavelength of 680 nm, and its electrophotographic performance was studied: E1/2 (light exposure necessary for lowering the charge to -350V) was 0.2  $\mu\text{J}/\text{cm}^2$  and the residual potential was -32V. The performance was found satisfactory.

A Canon-manufactured laser beam printer (LBP-8IV) was so modified as to give a spot ( $1/e^2$ ) having a diameter of 63.5  $\mu\text{m}$  in the subsidiary scanning direction, and of 20  $\mu\text{m}$  in the main scanning direction, to test the photosensitive member of this invention. The initial charging potential was set to -500V and the electrophotographic performance of the photosensitive member was studied. Its performance was satisfactory: after a 4,000 sheet running test, its wear was less than 0.1  $\mu\text{m}$ ; its angle in contact with water was 100°; its images suffered no notable deteriorations; and pixel reproducibility at highlighted portions was also good, in the face of input signals corresponding with 600 dpi.

## Comparative Example 2

5 Parts by weight of the triarylamine compound used in Example 1, and 5 parts by weight of a polycarbonate resin (tradename: Z-200, Mitsubishi Gas Chemicals) were dissolved into 70 parts by weight of chlorobenzene to produce a solution for charge transporting layer. This solution was applied through immersion coating onto the charge generating layer prepared in Example 2, and it was dried to form

## 26

a charge transporting layer of 10  $\mu\text{m}$  thickness. The resulting photosensitive member was evaluated in the same manner as in Example 2 above. A 4,000 sheet continuous running test revealed that its performance was poor: interference streaks and black dots appeared, the wear was as large as 1.8  $\mu\text{m}$ , it gave a small angle of 72° in contact with water; and the pixel reproducibility at highlighted portions of 600 dpi was poor and uneven.

## EXAMPLE 3

167 Parts by weight of a phenol resin (tradename: Plyophen, Dainippon Ink & Chemicals) were dissolved into 100 parts by weight of methylcellosolve, into which were dispersed 200 parts by weight of electroconductive barium sulfate ultra-fine particles (primary particle size being 50 nm). The mixture was applied through immersion coating onto the outer surface of an aluminum cylinder prepared as in Example 2 such that it gave, after being dried, a 10  $\mu\text{m}$  thick layer. Onto this electroconductive substrate were 20 formed a undercoat layer of 1  $\mu\text{m}$  thickness and a charge generating layer of 0.2  $\mu\text{m}$  thickness in the same manner as in Example 2.

Then, 40 parts by weight of organosilicon-modified triarylamine compound synthesized in Synthesis Example 8, 25 and 100 parts by weight of silicone thermosetting resin in Synthesis Example 2 were added to 100 parts by weight of toluene for dissolution. The mixture was further added with 0.5 part by weight of SiO<sub>2</sub> fine particles having an average diameter of 3  $\mu\text{m}$ . The blend was applied through immersion coating onto the charge generating layer. It was dried at 120° C. for 5 hours for thermal curing, to produce a charge transporting layer of 10  $\mu\text{m}$  thickness.

The specimen, when observed by microscopy, was transparent and uniform except for SiO<sub>2</sub> particles.

Its pencil hardness was 4H, and has an angle of 110° in contact with water.

This electrophotographic photosensitive member, after being charged with -700V, was exposed to light with a wavelength of 680 nm, and its electrophotographic performance was studied: E1/2 (light exposure necessary for lowering the charge to -350V) was 0.23  $\mu\text{J}/\text{cm}^2$  and the residual potential was 31V. The performance was found satisfactory.

The photosensitive member of this invention was applied to the same laser beam printer as used in Example 2 to be tested of its performance. The initial charging potential was set to -500V. Its performance was satisfactory: after a 10,000 sheet running test, the wear of the photosensitive member was extremely small, that is, 0.2  $\mu\text{m}$ ; its angle in contact with water was 102°, a satisfactory value; its images suffered no notable deteriorations such as black dots and interference streaks; and pixel reproducibility at highlighted portions was also good, in the face of input signals corresponding with 600 dpi.

## EXAMPLE 4

Layers up to a charge generating layer were formed in the same manner as in Example 1.

60 Then, to the same solution used to form a charge transporting layer in Example 1 added was 0.1 part by weight of silicone fine particles having an average diameter of 2  $\mu\text{m}$ , and the mixture was applied through immersion coating onto said charge generating layer to form, after being dried, a layer of 9  $\mu\text{m}$  thickness.

Then, to add a surface protecting layer, a curable composition produced by adding 200 parts by weight of toluene

and 40 parts by weight of 4-[N,N-bis(3,4-dimethylphenyl)amino]-[2-(triethoxysilyl)ethyl]benzene synthesized in Synthesis Example 8 to 100 parts by weight of the curable composition prepared in Synthesis Example 4, was applied through spray coating.

The assembly was allowed to dry at 140° C. for 4 hours, and a clear, even surface-protecting layer with a thickness of 3  $\mu\text{m}$  was formed thereupon after thermal curing. Its pencil hardness was 2H, and has an angle of 115° in contact with water.

The resulting electrophotographic photosensitive member was evaluated of its electrophotographic performance in the same manner as in Example 1: E1/2 was 0.70  $\mu\text{J}/\text{cm}^2$  and the residual potential was -35V. The performance was satisfactory.

The electrophotographic photosensitive member was applied to the same digital full-color copying machine as used in Example 1 to be evaluated of its imaging performance. The initial charging potential was set to -400V. A 10,000 sheet running test revealed that the photosensitive member was satisfactory in performance: its wear after the test was extremely small or 0.13  $\mu\text{m}$ ; its angle in contact with water was 109°; and it gave images excellent in reproducibility both at highlighted portions and at highly concentrated portions. Example 5

Layers up to a charge generating layer were formed in the same manner as in Example 2.

Then, 60 parts by weight of the organosiliconmodified triarylamine compound synthesized in Synthesis Example 13 and 100 parts by weight of the silicone heat curable resin in Synthesis Example 3 were added to 100 parts by weight of toluene for dissolution. The mixture was applied through immersion coating onto said charge generating layer. It was dried at 120° C. for 5 hours for thermal curing, to form a charge transporting layer of 10  $\mu\text{m}$  thickness. Thus, a photosensitive member of this invention was produced.

Its pencil hardness was 5H, and has an angle of 107° in contact with water.

It was evaluated of its electrophotographic performance in the same manner as in Example 2: E1/2 was 0.20  $\mu\text{J}/\text{cm}^2$  and the residual potential was -45V.

This photosensitive member was applied to the same laser beam printer as used in Example 2 to be tested of its performance. The initial charging potential was set to -500V. Its performance was satisfactory: after a 10,000 sheet running test, its wear was extremely small, that is, 0.28  $\mu\text{m}$ ; its angle in contact with water was 98°, a satisfactory value; its images suffered no notable flaws such as black dots and interference streaks; and pixel reproducibility at highlighted portions was also good, in the face of input signals corresponding with 600 dpi.

What is claimed is:

1. An electrophotographic photosensitive member comprising a substrate and a photosensitive layer thereupon, wherein a surface layer of the electrophotographic photosensitive member contains a resin which is obtained by curing a curable organosilicon polymer and an organosilicon-modified positive hole transporting compound as represented by the formula (I):



where A represents a positive hole transporting group, Q is a hydrolyzing group or hydroxyl group, R<sup>2</sup> is a substituted or unsubstituted monovalent hydrocarbon group, R<sup>3</sup> is a

substituted or unsubstituted alkylene or arylene group, "m" is an integer of 1 to 3, and "l" is a positive integer.

2. An electrophotographic photosensitive member according to claim 1, wherein R<sup>2</sup> is a monovalent hydrocarbon group with a carbon number of 1 to 15 or a halogen-substituted monovalent hydrocarbon group with a carbon number of 1 to 15, R<sup>3</sup> is -(CH<sub>2</sub>)<sub>n</sub>- (n is an integer of 1 to 18), and "l" is an integer of 1 to 5.

3. An electrophotographic photosensitive member according to claim 1, wherein Q is -OR<sup>1</sup> (R<sup>1</sup> represents an alkyl group or alkoxyalkyl group).

4. An electrophotographic photosensitive member according to claim 3, wherein R<sup>1</sup> has a carbon number of 1 to 6.

5. An electrophotographic photosensitive member according to claim 1, wherein A is represented by the following formula (II):



where R<sup>4</sup>, R<sup>5</sup> and R<sup>6</sup> are organic groups, at least one of them represents an aromatic hydrocarbon cyclic group or heterocyclic group, and R<sup>4</sup>, R<sup>5</sup> and R<sup>6</sup> may be the same, or different each other.

6. An electrophotographic photosensitive member according to claim 1, wherein a curable organosilicon polymer is represented by the following formula (III):



where R<sup>7</sup> represents a straight chain or branched alkyl group, alkenyl group or aryl group, R<sup>8</sup> is a hydrogen atom or an alkyl group, and r and s are molar ratios.

7. An electrophotographic photosensitive member according to claim 6, wherein r is 0.5 to 1.5 on the average and s is 0.01 to 1.5 on the average.

8. An electrophotographic photosensitive member according to claim 1, wherein the organosilicon-modified hole transporting compound has an ionizing potential of 4.5 to 6.2 eV.

9. An electrophotographic photosensitive member according to claim 1, wherein the organosilicon-modified hole transporting compound has a drift mobility of 1×10<sup>-7</sup> cm<sup>2</sup>/V.sec or more.

10. A process cartridge, comprising an electrophotographic photosensitive member, and at least one means selected from the group consisting of a charging means, a developing means and a cleaning means, wherein:

the electrophotographic photosensitive member and at least one means selected from the group are assembled into a unit which is reversibly set to the main body of an electrophotographic apparatus; and

electrophotographic photosensitive member, comprising a substrate and a photosensitive layer thereupon, wherein a surface layer of the electrophotographic photosensitive member contains a resin which is obtained by curing a curable organosilicon polymer and an organosilicon-modified positive hole transporting compound represented by the following formula (I):



where A represents a positive hole transporting group, Q is a hydrolyzing group or hydroxyl group, R<sup>2</sup> is a substituted or unsubstituted monovalent hydrocarbon group, R<sup>3</sup> is a substituted or unsubstituted alkylene group or arylene group, "m" is an integer of 1 to 3, and "l" is a positive integer.

**11.** A process cartridge according to claim **10**, wherein R<sup>2</sup> is a monovalent hydrocarbon group with a carbon number of 1 to 15 or a halogen-substituted monovalent hydrocarbon group with a carbon number of 1 to 15, R<sup>3</sup> is —(CH<sub>2</sub>)<sub>n</sub>— (n is an integer of 1 to 18), and “l” is an integer of 1 to 5.

**12.** An image forming apparatus, comprising an electrophotographic photosensitive member, a charging means, an exposure means, a developing means and a transferring means, wherein:

the electrophotographic photosensitive member comprises a substrate and a photosensitive layer thereupon, wherein a surface layer of the electrophotographic photosensitive member contains a resin which is obtained by curing a curable organosilicon polymer and an organosilicon-modified positive hole transporting compound represented by the following formula (I):



where A represents a positive hole transporting group, Q is a hydrolyzing group or hydroxyl group, R<sup>2</sup> is a substituted or unsubstituted monovalent hydrocarbon group, R<sup>3</sup> is a substituted or unsubstituted alkylene or arylene group, “m” is an integer of 1 to 3, and “l” is a positive integer.

**13.** An image forming apparatus according to claim **12**, wherein R<sup>2</sup> is a monovalent hydrocarbon group with a carbon number of 1 to 15 or a halogen-substituted monova-

lent hydrocarbon group with a carbon number of 1 to 15, R<sup>3</sup> is —(CH<sub>2</sub>)<sub>n</sub>— (n is an integer of 1 to 18), and “l” is an integer of 1 to 5.

**14.** An electrophotographic photosensitive member according to claim **1** or **2**, wherein m is 2 or 3.

**15.** A process cartridge according to claim **10** or **11**, wherein m is 2 or 3.

**16.** An image forming apparatus according to claim **12** or **13**, wherein m is 2 or 3.

**17.** An electrophotographic photosensitive member according to claim **1**, wherein the photosensitive layer is the surface layer.

**18.** A process cartridge according to claim **10**, wherein the photosensitive layer is the surface layer.

**19.** An image forming apparatus according to claim **12**, wherein the photosensitive layer is the surface layer.

**20.** An electrophotographic photosensitive member according to claim **1**, wherein the surface layer is a protective layer.

**21.** A process cartridge according to claim **10**, wherein the surface layer is a protective layer.

**22.** An image forming apparatus according to claim **12**, wherein the surface layer is a protective layer.

\* \* \* \* \*

UNITED STATES PATENT AND TRADEMARK OFFICE  
CERTIFICATE OF CORRECTION

PATENT NO. : 5,879,847

DATED : March 9, 1999

INVENTOR(S) : KAZUO YOSHINAGA, ET AL.

Page 1 of 2

It is certified that error appears in the above-identified patent and that said Letters Patent is hereby corrected as shown below:

On the title page:

AT [56] REFERENCES CITED

U.S. PATENT DOCUMENTS

"5,436,099 7/1995 Schank et al. 430/59" should be added.

COLUMN 7

Line 46, "positionis" should read --position is--.

COLUMN 9

Line 15, "each" should read --with each--.

COLUMN 11

Line 38, "or" should read --a--; and

Line 42, "or" should read --a--.

UNITED STATES PATENT AND TRADEMARK OFFICE  
CERTIFICATE OF CORRECTION

PATENT NO. : 5,879,847

DATED : March 9, 1999

INVENTOR(S) : KAZUO YOSHINAGA, ET AL.

Page 2 of 2

It is certified that error appears in the above-identified patent and that said Letters Patent is hereby corrected as shown below:

COLUMN 26

Line 20, "a" (first occurrence) should read --an--.

Signed and Sealed this

Seventh Day of December, 1999

Attest:



Q. TODD DICKINSON

Attesting Officer

Acting Commissioner of Patents and Trademarks